

## UNITED STATES PATENT OFFICE

MATHIAS PIER, OF HEIDELBERG, AND FRIEDRICH RINGER, OF LUDWIGSHAFEN-ON-THE-RHINE, GERMANY, ASSIGNEES, BY MESNE ASSIGNMENTS, TO STANDARD-I. G. COMPANY, OF LINDEN, NEW JERSEY, A CORPORATION OF DELAWARE

METHOD OF MAKING MOTOR FUELS

No Drawing. Application filed May 3, 1929, Serial No. 360,316, and in Germany May 21, 1928.

This invention relates to the manufacture and production of motor fuels.

The manufacture of non-knocking motor fuels, in particular of non-knocking gaso-lines, is of great technical importance. Hitherto attempts have been made to render motor fuels having a tendency to knock non-knocking by the addition of benzene or organic metallic compounds but these processes

10 have many drawbacks.

We have now found that in the produc-tion of motor fuels, the high-boiling frac-tions of hydrocarbon oils, boiling up to about 180° or 200° C. and above about 120° C. and 15 especially such fractions containing large amounts of compounds containing double bonds in the molecule are of extreme im-portance with regard to suppressing the knocking action of the said fuels. In accord-20 ance with the present invention non-knock-ing motor fuels are obtained by blending the said high-boiling anti-knocking frac-tions with low-boiling hydrocarbon frac-tions, usually boiling below about 150° C., 25 and usually or for the most part below 120° C., which by themselves have a tendency to knock, for example those containing mainly substances of the nature of paraffins. The addition of low-boiling hydrocarbons, poor 30 in hydrogen, such for example as benzene, for the prevention of knocking in motor fuels is already known, but the action of such anti-knocking agents is comparatively slight, so that it is necessary to add fairly large 35 quantities of the same to knocking benzines in order to prevent knocking, for example additions of 20 to 30 per cent of benzene and more, are necessary, whereas the same effect is produced by adding much smaller quanti-ties for example up to about 10 per cent of 40 the said higher boiling substances, in par-ticular those which are rich in hydrocarbons containing double bonds in the molecule such as aromatic or unsaturated hydrocarbons 45 and which boil between about 150° and 180° C. Additions of about 20 to 30 per cent of the said high-boiling fractions furnish par-ticularly valuable fuels, but in any case, so 50 much fuel is added that the knocking is sub-stantially suppressed.

We have further found that particularly valuable motor fuels are obtained if at least the said high-boiling non-knocking fraction is derived from the destructive hydroge-nation of hydrocarbon products, in particular 55 by the destructive hydrogenation of ali-phatic and hydroaromatic compounds, or by the destructive hydrogenation of aromatic middle oils, such as anthracene oils, mineral coal tar products, residue obtained by crack-ing, high temperature tars and the like. The motor fuels herein referred to, are of great importance because the low boiling and knocking constituents may be readily ob-tained by hydrogenation of aliphatic and hy-droaromatic compounds whilst the aromatic parent substances are easily converted into constituents boiling above 150° C. whereas 60 they are only difficultly converted into low-boiling constituents. 70

It is frequently the case that by destruc-tive hydrogenation, for example of middle oils, about 50 per cent of benzene containing many low-boiling constituents and compara-tively rich in hydrogen is easily obtained by 75 a single treatment for example by a treat-ment with hydrogen at 200 atmospheres and at about 450° C. The remaining 50 per cent may then be readily converted into hydrocar-bons, consisting of anti-knocking constitu-80 ents, a portion of which boils above 150° C. without any substantial loss of gas. By mix-ing these with the benzene obtained in the first treatment a non-knocking fuel is ob-tained, whereas if the initial materials had 85 been completely converted into benzene a knocking fuel might have been obtained.

The following examples will further illus-trate the nature of the invention but the in-vention is not restricted thereto. 90

*Example 1*

Straight-run gasoline from Pennsylvanian crude oil exhibits very considerable knock-ing when employed in an ordinary motor on account of its being practically exclusively composed of hydrocarbons of the paraffin series, so that even an addition of about 50 per cent by volume of benzene does not entirely 95 suppress knocking. If the said gasoline be 100

distilled and 3 parts of a fraction boiling up to 150° C. be mixed with 1 part of a fraction boiling substantially between 140° and 180° C. of a product obtained by treating 5 Coastal gas oil with hydrogen at about 560° C. and under a pressure of 200 atmospheres in the presence of a catalyst immune to sulfur poisoning, such as ferro-silicon, a motor fuel is obtained which is practically free from 10 knocking.

*Example 2*

Mid-Continent straight-run gasoline does not as a rule knock quite so much as Pennsylvanian gasoline. Very considerable additions of benzene, namely about 40 per cent by volume are, however, required in order to obtain a fuel which is passably free from knocking. If 4 parts by volume of those fractions of Mid-Continent gasoline boiling up to about 150° C. be mixed with a fraction boiling substantially between 145° and 185° C., obtained from well purified tar, derived from the carbonization of pit coal a motor fuel is obtained which even in motors having a high compression ratio shows no tendency to knocking.

*Example 3*

By the "topping" of a paraffinic American petroleum, for example Crane Upton crude oil, a gasoline is obtained which produces marked knocking in a motor under normal compression. By distilling off the fraction of this gasoline which boils below 150° C. 30 and making it with the same amount of a hydrocarbon fraction which is rich in aromatic constituents, which boils at between 150° and 180° C. and which has been obtained by destructive hydrogenation to obtain a normal 35 boiling point curve, a gasoline is obtained 40 which meets all requirements with regard to non-knocking.

What we claim is:—

The process of producing an anti-knock 45 fuel which comprises destructively hydrogenating aromatic middle oils by subjecting said oils to the action of hydrogen at a temperature of at least 450° C. a pressure of the order of 200 atmospheres and a catalyst immune to sulphur poisoning and then isolating 50 a fraction boiling between about 150 and 200° C. from the product so produced.

In testimony whereof we have hereunto set our hands.

MATHIAS PIER.  
FRIEDRICH RINGER.